

# UNITED STATES PATENT OFFICE.

CHARLES F. LINDSAY, OF FAIRFIELD, AND WALTER R. HIBBARD, OF BRIDGEPORT, CONNECTICUT, ASSIGNEES TO UNION METALLIC CARTRIDGE COMPANY, OF BRIDGEPORT, CONNECTICUT, A CORPORATION OF CONNECTICUT.

## PROCESS OF WATERPROOFING PAPER TUBES.

1,130,303.

Specification of Letters Patent.

Patented Mar. 2, 1915.

No Drawing.

Application filed May 28, 1914. Serial No. 841,529.

To all whom it may concern:

Be it known that we, (1) CHARLES F. LINDSAY, a subject of the King of Great Britain, and (2) WALTER R. HIBBARD, a citizen of the United States, residing at (1) Fairfield and (2) Bridgeport, county of Fairfield, State of Connecticut, have invented an Improved Process of Waterproofing Paper Tubes, of which the following is 10 a specification.

In the production of paper tubes, especially tubes which are intended for use in the manufacture of bodies for paper cartridge shells, it is desirable and necessary 15 that the tubes shall be of uniform diameter throughout; that the surface shall be waterproofed; and for commercial reasons, that the color shall appear the same, or nearly the same, over the entire outer surface of 20 the tubes.

The object of the present invention is to produce such tubes, and by employing the process hereinafter set forth, such object is accomplished.

25 The usual practice in making such tubes is to roll a sheet of paper into tubular form and stick the same with suitable adhesive. The tubes are dried, and after drying, they are lubricated, and by passing through suitable dies, they are polished and brought to exact size. Such tubes are then waterproofed by immersion in a bath of molten paraffin wax or other suitable waterproofing material.

35 Our invention relates specifically to the processes involved after the tube is rolled and dried, and before the tube is immersed in the paraffin bath. We have found, by repeated experiments, that, by coating the 40 dry and unsized paper tubes with polymerizable oils or suitable solutions or mixtures of polymerizable oils with other lubricants, such oils or mixtures serve as a very efficient lubricant, and at the same time, 45 after gelatinization, give a superior waterproofing to the tubes. It should be understood that the word "sizing" as herein used refers to the passage of the tubes through dies, or by other means bringing the tubes 50 to exact size. As is well known, these polymerizable oils may be gelatinized by various methods of which it is only necessary to mention here application of heat, exposure to air for considerable time, or treat-

ment with various chemical agents or gases. 55 For our purposes, we prefer heating the tubes to insure their gelatinization. Our invention, however, should not be so restricted, as we fully recognize that other methods of gelatinization may be used. In sizing the 60 tubes, the dies become heated by friction so that the polymerizable oil can be wholly or in part gelatinized by this process. We find in practice that our novel process gives a superior waterproofing without additional 65 treatment, but if preferred the tubes may be additionally immersed in paraffin or other waxes, and treated in the usual manner.

We have demonstrated that tubes, after 70 treatment with polymerizable oils and containing but a small percentage of their weight in oil, are as well waterproofed as tubes which have been impregnated with paraffin wax or by other processes, and 75 which contain sometimes upward of thirty per cent. of their weight in wax.

A very efficient treatment consists in surface treating the paper tubes with a solution of twenty parts of Chinese wood oil, 80 (tung oil), nine parts of carbon tetrachlorid, and one part of lubricating grease. Tubes, surface treated with this material, sized, and heated, are found to contain approximately two and one-half per cent. of their 85 weight of gelatinized Chinese wood oil and to be well waterproofed.

Having thus described our invention, we claim:

1. The process of waterproofing paper 90 tubes which consists in surface treating unsized tubes with a polymerizable oil, sizing the same by passage through suitable dies, and thereafter gelatinizing the polymerizable oil. 95

2. The process of waterproofing paper tubes which consists in coating the unsized tubes with a polymerizable oil, sizing the same, and gelatinizing the polymerizable oil by heat. 100

3. The process of waterproofing paper tubes which consists in treating the unsized paper tubes with a mixture of a polymerizable oil and other lubricant and thereafter sizing the same and by any suitable means 105 gelatinizing the polymerizable oil contained therein.

4. The process of waterproofing paper

2  
tubes which consists in surface coating the  
unsized tubes with a solution of Chinese  
wood oil substantially as described, sizing  
the same and gelatinizing the Chinese wood  
oil by immersion in a bath of molten wax.

5. The process of waterproofing paper  
tubes which consists in coating the same  
with a solution of Chinese wood oil, sizing,  
and heating the tubes to gelatinize the

Chinese wood oil contained therein, and  
thereafter impregnating with paraffin wax.

In testimony whereof we affix our signa-  
tures in presence of two witnesses:

CHARLES F. LINDSAY.  
WALTER R. HIBBARD.

Witnesses:

LENA M. JOHNSON,  
MARY S. BURROUGHS.